# EUROPEAN PATENT SPECIFICATION

(11) **EP 1 867 782 B1**
(45) Date of publication and mention of the grant of the patent: **15.07.2015**
(21) Application number: 06714979.9
(22) Date of filing: 01.03.2006
(51) Int. Cl.: A24D 1/02

(54) **LOW FLAME-SPREADING CIGARETTE PAPER**
ZIGARETTENPAPIER MIT LANGSAMER FLAMMENVORTRIEBSGESCHWINDIGKEIT
PAPIER DE CIGARETTE A FAIBLE PROPAGATION DU FEU

(30) Priority: 15.03.2005 JP 2005073055
(43) Date of publication of application: 19.12.2007
(73) Proprietor: Japan Tobacco Inc., Tokyo 105-8422 (JP)
(72) Inventor: KOMINAMI, Takashi, Tokyo 105-8422 (JP); MATSUFUJI, Takaaki, Tokyo 105-8422 (JP); UYAMA, Ken, Tokyo 105-8422 (JP)
(74) Representative: Isarpatent
(86) International application number: PCT/JP2006/303861
(87) International publication number: WO 2006/098153

(56) References cited:
- WO-A1-02/17737
- WO-A1-02/37991
- WO-A1-02/078471
- GB-A- 1 524 211
- US-A- 5 820 998
- US-A1- 2003 136 420

## Description

### Technical Field

The present invention relates to a low flame-spreading cigarette paper, and particularly, to a cigarette paper exhibiting both a low flame-spreading property and a low C/T ratio.

### Background Art

For example, a cigarette paper provided with bands formed of a flame retardant substance coated on a base cigarette paper is proposed (Jpn. Pat. Appln. KOKAI Publication No. 7-300795), in order to hardly cause the flame to spread from the kindling to, e.g., the floor when the cigarette is dropped on the floor through, for example, the carelessness of the smoker. This technique is based on the idea that when regions having a high combustibility and regions having a low combustibility are formed on a cigarette paper, the ordinary smoking can be performed at the region having a high combustibility, but, if a substance is brought into contact with the cigarette at the regions having a low combustibility, the cigarette is self-extinguished.

However, where a cigarette is manufactured by using the conventional low-flame spreading cigarette paper noted above, the carbon monoxide/tar ratio (C/T ratio) per cigarette is not sufficiently low.

WO 02/37991 discloses a cigarette paper exhibiting a low flame-spreading property, having a basis weight in the range of 15 to 40 g/m², a filler loading in the range of 10% to 40% by weight (i.e. 1.5 to 16 g/m²), and burn suppressing regions and discrete band coated regions, including alginate in an amount of about 1% to 20% by weight of the paper (i.e. 0.15 to 8 g/m² of the coated portion).

US 2003/136420 also discloses a cigarette paper exhibiting a low flame-spreading property having a total filler loading added to the paper wrapper in the range of about 10 to 40% by weight, a basis weight of cigarette wrapping paper between about 18 to 60 g, and burn suppressing regions and discrete band coated regions, including alginate. Several types and viscosities of alginates are described. Specific polymerization degrees of alginate are not mentioned.

### Disclosure of Invention

Therefore, it is an object of the present invention to provide a cigarette paper exhibiting a low flam-spreading property and achieving a low C/T ratio.

According to the present invention a cigarette paper is provided exhibiting a low flame-spreading property, comprising, on one surface of a base cigarette paper containing a filler in an amount of 2 to 6 g/m² and having a basis weight of 16 to 22 g/m², burn-suppressing regions coated with a burn-suppressing agent, provided spaced apart from each other, wherein a total coating amount of the burn-suppressing agent corresponds to 0.2 to 0.3 g per m² of the coated portion and wherein the burn-suppressing agent is sodium alginate having a degree of polymerization of 650 to 670, and wherein the base cigarette paper has an air permeability of 31 to 37 CORESTA.

### Brief Description of Drawings

The single figure is a schematic oblique view, partly broken away, exemplifying a construction of a cigarette wrapped with a cigarette paper according to one embodiment of the present invention.

### Best Mode for Carrying Out the Invention

The present invention will now be described in more detail.

In the cigarette paper of the present invention, burn-suppressing regions coated with a burn-suppressing agent are formed apart from each other on one surface of a base cigarette paper.

The base cigarette paper is based on an ordinary pulp such as flax pulp that is generally used for cigarette papers. However, the base cigarette paper contains a filler in an amount of 2 to 6 g/m², and has a basis weight of 16 to 22 g/m².

As the filler, use may be made of materials that are used generally including, for example, carbonates such as calcium carbonate and potassium carbonate, and hydroxides such as calcium hydroxide and magnesium hydroxide.

A burn adjusting agent such as citric acid or a salt thereof (sodium salt or potassium salt) may be added to the cigarette paper. These burn-adjusting agents, if added, may be used in an amount of up to 2% by weight in the base cigarette paper.

On one surface of the base cigarette paper, burn-suppressing regions, which are formed by coating of a burn-suppressing agent, are provided apart from each other. The burn-suppressing regions may be provided in the form of a plurality of stripes such that when a tobacco rod is wrapped with the cigarette paper, they extend in the longitudinal direction of the tobacco rod and are spaced apart from each other in the circumferential direction of the tobacco rod. Alternatively, the burn-suppressing regions may be provided in the form of a plurality of annular rings such that they extend in the circumferential direction of the tobacco rod and are spaced apart from each other in the longitudinal direction of the tobacco rod. In any case, the total coating amount of the burn-suppressing agent (dry basis) corresponds to 0.2 to 0.3 g/m² per m² of the coated region.

As the burn-suppressing agent, sodium alginate with a degree of polymerization of 650 to 670 is used. Sodium alginates having various degrees of polymerization are commercially available. Sodium alginate having such a high degree of polymerization exhibits a high burn-suppressing effect even when used in a small amount.

In the present invention, the low flame-spreading property and the low C/T ratio can be exhibited at the same time by setting the amount of the filler in the base cigarette paper, the basis weight of the base cigarette paper, and the total coating amount of burn-suppressing agent within the ranges described above.

The low flame-spreading cigarette paper of the present invention is used to wrap a tobacco rod formed of, for example, tobacco shreds, and generally, the surface on which the burn-suppressing agent is coated is brought into contact with the tobacco rod.

FIG. 1 illustrates a cigarette wrapped with a cigarette paper on which a burn-suppressing agent is coated in the form of annular rings.

Referring to FIG. 1, a cigarette 10 comprises a tobacco rod 11 consisting of a tobacco filler 13 that is wrapped with a base cigarette paper 12 in the form of a column. The base cigarette paper 12 has an inherent air permeability of 31 to 37 CORESTA units. In general, the tobacco rod 11 has a circumference of 17 to 26 mm and a length of 49 to 90 mm. An ordinary filter 18 may be attached to the proximal end portion (i.e., downstream edge portion in the inhaling direction) of the tobacco rod 11 by using a chip paper 17 according to the ordinary method.

An annular region 14 coated with a burn-suppressing agent is formed on the base cigarette paper 12, defining a burn-suppressing region. Where a plurality of annular burn-suppressing regions 14 are formed as illustrated in FIG. 1, these annular regions 14 are formed apart from each other in the longitudinal direction of the tobacco rod.

An ordinary burn region 15 that is not coated with a burn-suppressing agent is formed between adjacent annular burn-suppressing regions 14. Since the region 15 is constituted by a part of the base cigarette paper 12, it can burn under the ordinary smoking state like the base cigarette paper 12 itself. It follows that the region 15 acts as an ordinary burn region. For example, it is possible to form 1 to 3 annular burn-suppressing regions 14. Also, the annular burn-suppressing region 14 may have a width of 4 to 7 mm in the longitudinal direction and generally have a thickness of 0.1 to 5 µm. Where a plurality of burn-suppressing regions 14 are formed, distance between the adjacent burn-suppressing regions 14 is preferably 18 to 25 mm.

In the cigarette shown in FIG. 1, a region 16 covering a distance d from the tip is not coated with a burn-suppressing agent. This section at the tip portion, which is not coated with the burn-suppressing agent, also constitutes an ordinary burn region, and can correspond to the region that is combusted by one puff or two puffs in the ordinary cigarette. Incidentally, where a plurality of burn-suppressing regions 14 are provided, the ordinary burn region 16 may not be formed (d = 0). However, where a single burn-suppressing region 14 is provided, the distance d from the tip 11a of the tobacco rod can be set at 10 to 25 mm. It is not particularly necessary to form a burn-suppressing region 14 on the inner surface of the cigarette paper corresponding to that portion of the cigarette paper 12 which is covered with the chip paper 17.

When the cigarette 10 is ignited at the tip 11a and inhaled to be burnt, the cigarette can burn at the ordinary burn region 15 like an ordinary cigarette and the flavor and taste can be enjoyed. However, if the cigarette 10 under the ignited state is put on a combustible material such as a carpet, a tatami mat, a wooden article, cloths, or clothing, the burn-suppressing region 14 extending in the combusting direction, the heat absorption by the combustible substance, and the expanded tobacco shreds collectively serve to extinguish the cigarette 10, and prevent the combustible substance from catching fire. Also, the cigarette wrapped with the cigarette paper of the present invention is low in the C/T ratio in the mainstream smoke.

The present invention will be described by way of Examples below. However, the present invention is not limited by these Examples.

### Examples 1 to 3 and Comparative Examples 1 to 22

A base paper (width 27 mm; length 1.500m) of the specification shown in Table 1 was coated (printed) with an aqueous solution of sodium alginate of various concentrations (0.5 to 20% by weight) at a constant width of 7 mm in the longitudinal direction and a constant spacing of 20 mm in the form of stripes by a direct gravure method, forming a total of 56 burn-suppressing agent-coated regions. For the cigarette paper thus obtained, the total coating amount of sodium alginate was measured according to the procedures described below. The results are shown also in Table 1. As shown in Table 1, the total coating amount of the burn-suppressing agent per m² of the region coated with the burn-suppressing agent (sodium alginate) corresponded to 0.2 to 1.8g in the papers of the Examples and the Comparative Examples. This coating amount of the burn-suppressing agent can be converted to the amount of the burn-suppressing agent per area of the cigarette paper by being multiplied by 7/27, yielding 0.05 to 0.47 g/m², Incidentally, sodium alginate used in each of Examples 1, 2 and 3 was I-S manufactured by KIMIKA (registered trademark) (polymerization degree: 650 to 670; viscosity of its 3% by weight aqueous solution at 25°C: 29976.9 cP), and sodium alginate used in the Comparative Examples was IL-2 manufactured by KIMIKA (registered trademark) (polymerization degree: 30 to 180; viscosity of its 3% by weight aqueous solution at 25°C: 907.2 cP).

A tobacco rod consisting of American blend of tobacco shreds (tar amount without a filter: 19 to 20 mg) was wrapped with the cigarette paper obtained above, and was cut such that the first coated region was arranged 5 mm spaced apart from the burn edge of the cigarette. Each cigarette was 59 mm long, and had two burn-suppressing agent-coated regions.

The cigarette thus obtained was subjected to a burn test in accordance with ASTM E-2187-04 so as to measure the value of PFLB (percent full-length burn). Also, the CO amount in the mainstream smoke, the number of puffs and the tar amount for each cigarette sample were measured by the methods described below in respect of these cigarette samples. The results are shown in Table 2.

### <Measurement of Total Coating Amount of Sodium Alginate>

Measurement was made as follows in accordance with "Quantitative Analytical Method of Sodium Alginate in Food" described in "Food Hygienics Magazine", Vol. 5, pp. 297-302 (1988), without carrying out the degreasing, the treatment with a dilute sulfuric acid, and the protein-removing treatment.

The cigarette paper coated with the burn-suppressing agent (1.5000m; width 27 mm) (about 1.0g) was cut into pieces each sized at 5 mm square. Then, 40 mL of a 1% by weight aqueous solution of sodium hydrogen carbonate was added thereto, and heated for 5 minutes in a warm water bath at 60°C. Then, the mixture was sufficiently mixed, stirred, and subjected to centrifugal separation (3,500 rotations, 10 minutes; the same applies to the following) to give a supernatant liquor (extracted liquid). The extraction residue was similarly subjected again to the extraction to give a supernatant liquor (extracted liquid). In addition, 20 mL of a 1% by weight aqueous solution of sodium hydrogen carbonate was added to and mixed sufficiently with the extraction residue to give supernatant liquor (extracted liquid). These three extracted liquid were combined, and a 1% by weight aqueous solution of sodium hydrogen carbonate was added to 100 mL, which was used as a test solution.

2 mL of copper-hydrochloric acid solution (8.5M hydrochloric acid containing 0.05% by weight of copper sulfate) and 1 mL of a naphtoresorcinol solution (0.4% by weight aqueous solution of 1,3-dihydroxynaphthalene) were added to each of 1 mL of a sodium alginate standard solution (1% by weight aqueous solution of sodium hydrogen carbonate containing sodium alginate at a concentration of 0 to 0.2 mg/mL) and 1 mL of the test solution noted above. Then, each mixture was heated for 65 minutes in a boiling water bath, and then cooled in ice water, to which 4 mL of butyl acetate was added. The mixture was shaken and subjected to centrifugal separation.

1 mL was taken from the supernatant liquor after the centrifugal separation, diluted by adding 3 mL of butyl acetate and subjected to a colorimetric at 566 nm, and the total coating amount was calculated.

### <Measurement of CO Amount and the Number of Puffs>

For measuring the CO amount, the tobacco smoke was collected by using an 8-port linear smoking machine (SM 342) manufactured by FILTRONA Inc. For the burn of the cigarette, the suction of 35 mL/2 seconds was carried out at an interval of 60 seconds according to the ISO standards, and the smoke passing through the glass fiber filter was collected in a gas bag. The suction of the cigarette sample was stopped when the sample reached the standard burn length (51 mm from the ignition edge of the cigarette (8 mm apart from the tip side as measured from the boundary between the cigarette paper and the chip paper)). The number of puffs at this point was counted and recorded. After the burning, the igniting portion was removed and, then, blank puffing was performed three times so as to collect the gas remaining in the cigarette. In this fashion, the gas of the cigarette sample was collected in the gas bag, and the total particulate matter (TPM) was collected at the glass fiber filter.

The CO amount per cigarette sample was measured with a CO measuring apparatus manufactured by FILTRONA Inc., using the gas collected in the gas bag and

### <Measurement of Tar Amount>

From the particulate components collected at the glass fiber filter in measuring the CO amount, the crude tar amount was weighed, and then the filter was put in a serum bottle and vigorously shaken together with 10 mL of 2-propanol (GC grade, manufactured by Wako Junyaku K.K.). The extracted liquor was filtered and poured into a vial. Then, the extracted liquor was applied to a chromatograph so as to measure the water amount and the nicotine amount. The quantitative determination was carried out by the internal standard method, and the tar amount was obtained by subtracting the water amount and the nicotine amount from the crude tar amount

**Table 1: Specification of cigarette paper**

| Example | Base cigarette paper | | | | Total coating amount of burn-suppressing agent (g/m²) |
|---|---|---|---|---|---|
| | Filler (g/m²) | Basis weight (g/m²) | Burn-adjusting agent (% by weight) | Air permeability (CORESTA) | |
| Comp. Ex. 1 | 7.7 | 25 | 0.3 | 35 | 0 |
| Comp. Ex. 2 | 5.2 | 21 | 0.3 | 45 | 0 |
| Comp. Ex. 3 | 4.1 | 21 | 0.3 | 35 | 0 |
| Comp. Ex. 4 | 2.5 | 20 | 0.3 | 37 | 0 |
| Comp. Ex. 5 | 2.1 | 19 | 0.3 | 31 | 0 |
| Comp. Ex. 6 | 7.7 | 26 | 0.3 | 35 | 1.8 |
| Comp. Ex. 7 | 7.7 | 26 | 1.0 | 35 | 1.8 |
| Comp. Ex. 8 | 7.7 | 26 | 0.3 | 35 | 2.2 |
| Comp. Ex. 9 | 7.7 | 26 | 1.0 | 35 | 2.2 |
| Comp. Ex. 10 | 2.1 | 19 | 0.3 | 31 | 2.3 |
| Comp. Ex. 11 | 2.1 | 26 | 0.3 | 32 | 0.5 |
| Comp. Ex. 12 | 5.2 | 21 | 0.3 | 45 | 2.0 |
| Comp. Ex. 13 | 5.2 | 21 | 0.3 | 45 | 0.3 |
| Comp. Ex. 14 | 5.2 | 21 | 0.3 | 45 | 1.2 |
| Comp. Ex. 15 | 5.2 | 21 | 0.3 | 45 | 1.6 |
| Comp. Ex. 16 | 5.2 | 21 | 0.3 | 45 | 1.8 |
| Ex. 1 | 4.1 | 21 | 0.3 | 35 | 0.3 |
| Comp. Ex. 17 | 4.1 | 21 | 0.3 | 35 | 1.0 |
| Comp. Ex. 18 | 4.1 | 21 | 0.3 | 35 | 1.8 |
| Ex. 2 | 2.5 | 21 | 0.3 | 37 | 0.2 |
| Comp. Ex. 19 | 2.5 | 20 | 0.3 | 37 | 0.7 |
| Comp. Ex. 20 | 2.5 | 20 | 0.3 | 37 | 1.8 |
| Ex. 3 | 2.1 | 19 | 0.3 | 31 | 0.2 |
| Comp. Ex. 21 | 2.1 | 19 | 0.3 | 31 | 0.6 |
| Comp. Ex. 22 | 2.1 | 19 | 0.3 | 31 | 1.0 |

**Table 2: Test results**

| Example | PFLB (%) | Tar amount per cig. (mg) | CO amount per cig. (mg) | C/T ratio | Puff number | Remarks |
|---|---|---|---|---|---|---|
| Comp. Ex. 1 | 100 | 19.6 | 16.0 | 0.82 | 7.4 | |
| Comp. Ex. 2 | 81-95 | 21.0 | 15.2 | 0.72 | 7.6 | |
| Comp. Ex. 3 | 87-99 | 21.8 | 16.0 | 0.73 | 7.8 | |
| Comp. Ex. 4 | 81-95 | 23.2 | 16.2 | 0.70 | 8.1 | |
| Comp. Ex. 5 | 20-40 | 23.7 | 16.8 | 0.71 | 8.2 | |
| Comp. Ex. 6 | 20-40 | 21.1 | 18.4 | 0.87 | 8.2 | |
| Comp. Ex. 7 | 20-40 | 21.2 | 19.3 | 0.91 | 8.4 | |
| Comp. Ex. 8 | 0-5 | 21.6 | 19.0 | 0.88 | 8.4 | |
| Comp. Ex. 9 | 0-5 | 21.1 | 19.2 | 0.91 | 8.2 | |
| Comp. Ex. 10 | 0-5 | - | - | - | - | Impossible to measure; the cigarette went out |
| Comp. Ex. 11 | 0-5 | 22.9 | 20.6 | 0.90 | 8.5 | |
| Comp. Ex. 12 | 0-5 | - | - | - | - | Impossible to measure; the cigarette went out |
| Comp. Ex. 13 | 0-5 | 21.4 | 15.6 | 0.73 | 7.8 | |
| Comp. Ex. 14 | 0-5 | 22.3 | 16.5 | 0.74 | 8.2 | |
| Comp. Ex. 15 | 0-5 | 22.8 | 17.0 | 0.75 | 8.4 | |
| Comp. Ex. 16 | 0-5 | 23.0 | 17.2 | 0.75 | 8.5 | |
| Ex. 1 | 0-5 | 22.0 | 16.3 | 0.74 | 7.9 | |
| Comp. Ex. 17 | 0-5 | 23.0 | 17.4 | 0.76 | 8.4 | |
| Comp. Ex. 18 | 0-5 | 23.5 | 17.9 | 0.76 | 8.6 | |
| Ex. 2 | 0-5 | 23.4 | 16.4 | 0.70 | 8.2 | |
| Comp. Ex. 19 | 0-5 | 23.8 | 16.8 | 0.71 | 8.4 | |
| Comp. Ex. 20 | 0-5 | 25.1 | 18.1 | 0.72 | 9.0 | |
| Ex. 3 | 0-5 | 25.0 | 17.8 | 0.71 | 8.7 | |
| Comp. Ex. 21 | 0-5 | 25.3 | 18.2 | 0.72 | 8.9 | |
| Comp. Ex. 22 | 0-5 | 25.9 | 18.8 | 0.73 | 9.1 | |

From the results shown in Table 2, it can be seen that the cigarette papers (Examples 1-3) in which a burn-suppressing agent is coated spaced from each other on a base cigarette paper containing a filler in an amount of 2 to 6 g/m² and having a basis weight of 16 to 22 g/m² such that the total coating amount corresponds to 0.2 to 0.3 g/m² and wherein the burn suppressing-agent is sodium alginate with a polymerization degree of 650 to 670, and wherein the base cigarette paper has an air permeability of 31 to 37 CORESTA, exhibits a low flame-spreading property and a low C/T ratio.

As has been described above, the present invention provides a cigarette paper which exhibits a low flame-spreading property and achieves a low C/T ratio.

## Claims

1. A cigarette paper exhibiting a low flame-spreading property, comprising, on one surface of a base cigarette paper containing a filler in an amount of 2 to 6 g/m² and having a basis weight of 16 to 22 g/m², burn-suppressing regions coated with a burn-suppressing agent, provided spaced apart from each other, wherein a total coating amount of the burn-suppressing agent corresponds to 0.2 to 0.3 g per m² of the coated portion and wherein the burn-suppressing agent is sodium alginate having a degree of polymerization of 650 to 670, and wherein the base cigarette paper has an air permeability of 31 to 37 CORESTA.

2. The cigarette paper according to claim 1, wherein the burn-suppressing regions are in a form of a plurality of stripes such that when a tobacco rod is wrapped with the cigarette paper, they extend in a longitudinal direction of the tobacco rod and are spaced apart from each other in a circumferential direction of the tobacco rod.

3. The cigarette paper according to claim 1, wherein the burn-suppressing regions are in a form of a plurality of annular rings such that when a tobacco rod is wrapped with the cigarette paper, they extend in a circumferential direction of the tobacco rod and are spaced apart from each other in a longitudinal direction of the tobacco rod.

## Patentansprüche

1. Zigarettenpapier, das sich durch eine niedrige Flammausbreitungsgeschwindigkeit auszeichnet und das auf einer Fläche eines Basiszigarettenpapiers, das einen Füllstoff in einer Menge von 2 bis 6 g/m² enthält und ein Basisgewicht von 16 bis 22 g/m² besitzt, Brennunterdrückungsregionen umfasst, die mit einem Brennunterdrückungsmittel beschichtet sind und die in einem Abstand voneinander angeordnet sind, wobei eine Gesamtbeschichtungsmenge des Brennunterdrückungsmittels 0,2 bis 0,3 g je m² des beschichteten Abschnitts entspricht und wobei das Brennunterdrückungsmittel Natriumalginat ist, das einen Polymerisationsgrad von 650 bis 670 aufweist, und wobei das Basiszigarettenpapier eine Luftdurchlässigkeit von 31 bis 37 CORESTA aufweist.

2. Zigarettenpapier nach Anspruch 1, wobei die Brennunterdrückungsregionen in Form mehrerer Streifen dergestalt ausgebildet sind, dass sie sich, wenn ein Tabakstäbchen mit dem Zigarettenpapier umhüllt wird, in einer Längsrichtung der Tabakstäbchen erstrecken und in einer Umfangsrichtung des Tabakstäbchens voneinander beabstandet sind.

3. Zigarettenpapier nach Anspruch 1, wobei die Brennunterdrückungsregionen in Form mehrerer Ringe dergestalt ausgebildet sind, dass sie sich, wenn ein Tabakstäbchen mit dem Zigarettenpapier umhüllt wird, in einer Umfangsrichtung der Tabakstäbchen erstrecken und in einer Längsrichtung des Tabakstäbchens voneinander beabstandet sind.

## Revendications

1. Papier de cigarette présentant une propriété de faible propagation de flammes, comprenant, sur une surface d'un papier de cigarette de base contenant une charge dans une quantité de 2 à 6 g/m² et présentant une masse basique de 16 à 22 g/m², des régions supprimant la combustion revêtues avec un agent supprimant la combustion, fournies espacées les unes des autres, dans lequel une quantité totale de revêtement de l'agent supprimant la combustion correspond à de 0,2 à 0,3 g par m² de la portion revêtue et dans lequel l'agent supprimant la combustion est de l'alginate de sodium présentant un degré de polymérisation de 650 à 670, et dans lequel le papier de cigarette de base présente une perméabilité à l'air de 31 à 37 CORESTA.

2. Papier de cigarette selon la revendication 1, dans lequel les régions supprimant la combustion sont dans la forme de plusieurs bandes telles que, lorsqu'une tige de tabac est enveloppée avec le papier de cigarette, elles s'étendent dans une direction longitudinale de la tige de tabac et elles sont espacées les unes des autres dans une direction circonférentielle de la tige de tabac.

3. Papier de cigarette selon la revendication 1, dans lequel les régions supprimant la combustion sont dans une forme de plusieurs anneaux annulaires telles que, lorsqu'une tige de tabac est enveloppée avec le papier de cigarette, elles s'étendent dans une direction circonférentielle de la tige de tabac et elles sont espacées les unes des autres dans une direction longitudinale de la tige de tabac.
